

[54] ELECTROLYSIS OF ALKALI METAL CHLORIDES

[75] Inventors: **Karl Opp**, Heidelberg; **Ewald Wygasch**, Ludwigshafen; **Gotthard Csizi**, Bad Duerkheim, all of Germany

[73] Assignee: **Badische Anilin & Soda-Fabrik Aktiengesellschaft**, Ludwigshafen/Rhein, Germany

[22] Filed: **Apr. 21, 1971**

[21] Appl. No.: **136,213**

[30] Foreign Application Priority Data

Apr. 27, 1970 Germany ..... P 20 20 480.2

[52] U.S. Cl. .... **204/99, 204/140**

[51] Int. Cl. .... **C01d 1/08 C23b/1/00**

[58] Field of Search..... **204/99, 128, 140**

[56]

References Cited

UNITED STATES PATENTS

3,639,118 2/1972 O'Grady ..... 204/140 X  
3,364,128 1/1968 Williston et al..... 204/140

Primary Examiner—John H. Mack

Assistant Examiner—D. R. Valentine

Attorney—Johnston, Root, O'Keeffe, Keil, Thompson & Shurtleff

[57]

ABSTRACT

Disturbances occurring in chloride-caustic cells using the amalgam method are caused by felty coatings which form on the bottom of the cells. These disturbances can be avoided by treating the mercury (after it has left the decomposer and before or after it has entered the electrolytic cell) with an aqueous solution which contains chlorine and/or ferric chloride.

4 Claims, No Drawings

## ELECTROLYSIS OF ALKALI METAL CHLORIDES

In the electrolytic production of chlorine and an alkali metal hydroxide by the mercury method, cells are used whose bottom consists of iron and which must be covered completely with mercury. In order to achieve this, the bottom is amalgamated prior to setting the cell in operation so that it is made wettable by mercury and complete covering of the bottom is achieved even when the layer of mercury is not very thick. The covering of mercury is essential during operation of the cell because of the risk of the formation of hydrogen.

On the other hand, for reasons of keeping the consumption of energy at a minimum, the cell potential should be at an optimum low, i.e. the distance between the anodes and the mercury film should be as small and above all as uniform as possible. It is unfavorable if, owing to local variations in the thickness of the mercury layer, the mean distance between anode and cathode has to be markedly increased. Such an uneven distribution of mercury may result in the mercury film being split apart and then hydrogen will be formed as mentioned above. In chlorine-caustic cells as designed according to the present state of the art the two disturbances outlined above are caused by the deposition of traces of iron in the mercury. Iron is of course insoluble in mercury but forms a suspension of fine crystals of iron in the mercury. These particles are retained in the cell by magnetic forces so that after a few weeks' operation a felty coating forms on the bottom of the cell. Short-circuits occur owing to the local retention of mercury thus caused and it is necessary to raise the anodes. This increase in the mean distance between the electrodes causes an increase in the cell potential. The latest remedy for this is to open the cells at regular intervals of 6 to 8 weeks and to remove the iron amalgam mechanically from the bottom. This operation not only causes considerable assembly costs but also considerable losses in output.

In order to obviate this difficulty, attempts have been made to incline the cells more steeply in the hope that the mercury would flow sufficiently rapidly to carry the iron with it. This hope has only been partly realized because the thin layer of mercury cannot be accelerated beyond a certain extent even at a very great inclination. Moreover the magnetic forces also become greater as the current densities are increased. The said effect can be delayed by the said measures but cannot be prevented.

The present invention has as an object the prevention of the felty coating on the bottom of the cells in the electrolysis of alkali metal chlorides according to the amalgam process.

We have found that the said object is achieved in the electrolysis of alkali metal chlorides by treating the mercury (after the alkali metal amalgam has been destroyed) with an aqueous solution containing chlorine and/or ferric chloride.

Treatment of the mercury according to this invention is carried out after it has left the decomposer and before it enters the electrolytic cell or inside the latter. It may be carried out for example in packed towers into which the two liquids (mercury and the solution containing chlorine or ferric chloride) are introduced. The treatment may also be carried out inside the electrolytic cell itself, for example by appropriate subdivision of the same.

Since intense mixing of the two liquids is not necessary for the removal of iron from the mercury, however, it is possible according to a preferred embodiment of the invention to carry out the treatment of the mercury by providing a covering of the abovementioned oxidizing liquids over the mercury. This may be carried out for example by allowing the mercury from the decomposer to pass along a channel into which the aqueous solution is fed. For a given amount of mercury being circulated, the amount of aqueous solution fed in is such that by its content of active chlorine and/or ferric chloride, the iron content of the mercury for a given residence time does not fall below 0.01 percent by weight. If the treatment is carried further, there is a risk that mercury may be dissolved in appreciable quantities. Provided that the iron content in the recycled mercury is not allowed to rise above about 0.01 to 0.02 percent by weight, the felt formation referred to above can be reliably avoided. The duration of the treatment according to the invention will naturally depend on the amount of mercury to be treated and thus depends on the size of the electrolytic cell. It amounts as a rule to 1 to 10 percent of the residence time of the mercury in the electrolytic cell.

Chlorine-containing brine having the highest possible content of active chlorine is advantageously used as the chlorine-containing liquid. Iron chloride is also used in the form of a solution of the highest possible concentration to which it is advantageous to add from 0.5 to 5% by weight of HCl.

The following Example illustrates the invention.

## EXAMPLE

a. 4 cubic meters per hour of mercury (54.4 metric tons) is circulated through a 100 kiloampere mercury cell. Mercury leaving the decomposer has an iron content of 0.016% by weight. Prior to reentry into the electrolytic cell, the mercury is treated with 16 cubic meters per hour of a chlorine-containing sodium chloride brine having a content of active chlorine of 340 mg/l by covering it therewith in a channel having a length of 5 meters (residence time 22 seconds).

At the end of the channel the mercury is drawn off with an iron content of 0.012% by weight. The chlorine content of the brine has been decreased to 50 mg of active chlorine per liter.

The cell can be operated for months at a time without the occurrence of the disturbances described above.

b. The same results as regards the iron content of the mercury are achieved under otherwise the same conditions as under (a) by using 200 liters per hour of a ferric chloride solution containing hydro-chloric acid (pH = 2) and having a content of 40 g of  $Fe^{+++}$  per liter. The aqueous solution contains about 18 g of  $Fe^{+++}$  per liter and 32.88 g of  $Fe^{+++}$  per liter after the treatment.

We claim:

1. A process for the electrolysis of an alkali metal chloride by the amalgam method in a cell having a mercury cathode, decomposition of the alkali metal amalgam thus formed in a decomposer cell into mercury and caustic alkali solution and return of the mercury to the electrolytic cell wherein after the decomposition of the alkali metal amalgam the resultant mercury is treated with an aqueous solution which contains chlorine and/or ferric chloride, said treatment being controlled so that the iron content of the mercury is not decreased below 0.01% by weight.

2. A process as claimed in claim 1 wherein the treatment is carried out by covering the mercury with a layer of the aqueous solution.

3. A process as claimed in claim 1 wherein recycled mercury flows through a channel to which the aqueous

solution is supplied so that it covers the mercury.

4. A process as set forth in claim 1 wherein said aqueous solution contains ferric chloride.

\* \* \* \* \*